

## UNITED STATES PATENT OFFICE

2,211,912

## PREPARATION OF PIGMENTED COATINGS

Patrick J. Ryan, Royal Oak, Mich., assignor, by  
mesne assignments, to Reichhold Chemicals,  
Inc., Detroit, Mich., a corporation of Delaware

No Drawing. Application May 9, 1938,  
Serial No. 206,923

1 Claim. (Cl. 260—40)

The invention relates to improved pigmented coatings and to the method of preparing the same.

The conventional method for preparation of 5 pigmented coatings consists in wetting and dispersing a pigment in an organic solvent solution of a film forming material, such as mixtures of drying oils and synthetic resins.

Among the objects of my invention are to obtain 10 better wetting and dispersion of pigments, higher original gloss, superior gloss retention, better original color and better color retention, than is obtainable by conventional methods now in use. Another object is to shorten the time required for processing.

It is known that good gloss in coatings depends almost exclusively upon proper wetting and dispersion of pigments. This gloss is obtained by present methods by long grinding and mixing in pebble mills or by repeated passes 20 through a roller mill or stone mill. The purpose of this long grinding time is to obtain satisfactory wetting and dispersion of the pigment agglomerates by mechanical means. The word "grinding" is used throughout the industries to 25 designate wetting and dispersion of pigments in various vehicles and that word has been retained in this application to designate such and not to indicate a reduction of particle size of the pigments used. Pebble mills are considered to have 30 advantages over roller mills and stone mills insofar as no volatile losses are incurred during the processing, but it usually requires long periods of processing in a pebble mill before satisfactory gloss is obtained. Hence, many in the 35 industries have abandoned it in favor of the roller mill or stone mill.

My invention comprises pre-wetting and at 40 least partially dispersing pigments in suitable organic solvents for the film forming agent to be subsequently added and then introducing film forming substances into said mixture and applying sufficient mechanical forces to complete the dispersion. The employment of my invention 45 has decreased the "grinding" time of pigmented coatings from one-half to two-thirds the time normally used when processed by conventional method.

The process may be carried out without necessarily 50 employing super atmospheric pressure,

vacuum or increased temperature, though it will be understood that any of these factors may be present if desired, or if necessary in specific cases. The process may also be carried out without the loss of the volatiles used.

The invention will be more readily understood by reference to the following specific examples which are set forth by way of illustration and not by way of limitation:

## Example I

|                                 | Parts by weight |
|---------------------------------|-----------------|
| Titanium dioxide                | 950             |
| Zinc oxide                      | 50              |
| High solvency petroleum naphtha | 270 15          |

The above was charged into a pebble mill and tumbled for 10-15 minutes and the following was added:

|             | Parts by weight |
|-------------|-----------------|
| Vehicle (A) | 450             |

The mill was then tumbled for 72 hours and the following added:

|                                 | Parts by weight |
|---------------------------------|-----------------|
| Vehicle (A)                     | 1150            |
| High solvency petroleum naphtha | 302             |

The enamel prepared in this way was compared to one prepared by the following conventional method:

|                                 | Parts by weight |
|---------------------------------|-----------------|
| Titanium dioxide                | 950             |
| Zinc oxide                      | 50              |
| High solvency petroleum naphtha | 270 35          |
| Vehicle (A)                     | 450             |

The above was charged into the pebble mill in one operation and tumbled for 72 hours and the following was added:

|                                 | Parts by weight |
|---------------------------------|-----------------|
| Vehicle (A)                     | 1150            |
| High solvency petroleum naphtha | 302             |

Baked films of the enamels prepared according to my invention had superior gloss and color when freshly prepared, and after aging for six months in the dark, the gloss and color were far superior.

Vehicle (A) used in the experiment is a glyc-

5

10

20

25

30

35

40

45

50

erol phthalate soya bean fatty acid modified resin, dissolved in equal parts by weight of xylol.

Table I

|    | Coating                                                                                                                      | Tumbled hours | Comparison of degree of gloss |    |
|----|------------------------------------------------------------------------------------------------------------------------------|---------------|-------------------------------|----|
| 5  | Parts by weight                                                                                                              |               |                               | 5  |
|    | Titanium dioxide                                                                                                             | 1425          | 24 Less.                      |    |
|    | Zinc oxide                                                                                                                   | 75            | 32 More.                      |    |
|    | High solvency petroleum naphtha                                                                                              | 420           | 48 Do.                        |    |
| 10 | Parts by weight                                                                                                              |               | 56 Do.                        | 10 |
| 10 | The above was tumbled for 10-15 minutes in a pebble mill and the following was added:                                        |               | 72 Do.                        |    |
| 15 | Vehicle (A)                                                                                                                  | 630           | 80 Do.                        |    |
| 15 | The above was tumbled for the hours shown in Table I, and the following was added at the end of the time shown in the table: |               | 96 Do.                        |    |
| 20 | Parts by weight                                                                                                              |               | 104 Do.                       | 20 |
|    | Vehicle (A)                                                                                                                  | 1010          | 120 Do.                       |    |
|    | High solvency petroleum naphtha                                                                                              | 350           |                               |    |
| 25 | The coatings prepared in the above manner were compared to coatings prepared as follows:                                     |               |                               | 25 |
| 30 | Parts by weight                                                                                                              |               |                               | 30 |
|    | Titanium dioxide                                                                                                             | 1425          | 24 Less.                      |    |
|    | Zinc oxide                                                                                                                   | 75            | 32 Do.                        |    |
| 30 | High solvency petroleum naphtha                                                                                              | 420           | 48 Do.                        | 35 |
|    | Vehicle (A)                                                                                                                  | 630           | 56 Do.                        |    |
| 35 | The above was tumbled for the hours shown in Table I, and the following was added at the end of the time shown in the table: |               | 72 Do.                        |    |
|    | Parts by weight                                                                                                              |               | 80 Do.                        |    |
|    | Vehicle (A)                                                                                                                  | 1010          | 96 Used as standard.          |    |
|    | High solvency petroleum naphtha                                                                                              | 350           | 104 Equal.                    |    |
|    |                                                                                                                              |               | 120 Do.                       |    |

It is to be noted that the pigments, solvents and vehicle were all from the same source. The films were applied in the same manner, and baked at the same schedule, the only difference being in the preparation of the coatings as described.

I claim:

A process for preparing a liquid coating composition which comprises pre-wetting and partially dispersing an initially dry pigment in a relatively minor quantity of a volatile petroleum hydrocarbon in the absence of any film-forming agent, then grinding the same with a vehicle comprising a fatty acid modified glycerol phthalate resin dissolved in xylol until dispersion is substantially complete, and subsequently adding an additional quantity of the vehicle together with a further quantity of the volatile petroleum hydrocarbon.

PATRICK J. RYAN.